

[54] SILICATED SODA ASH

[75] Inventor: **Ralph E. Temple**, Chardon, Ohio

[73] Assignee: **Diamond Shamrock Corporation**,  
Cleveland, Ohio

[22] Filed: **May 3, 1972**

[21] Appl. No.: **250,031**

[52] U.S. Cl. .... **252/135, 252/385**

[51] Int. Cl. .... **C11d 3/08, C11d 3/10**

[58] Field of Search. .... **252/135, 385, 99**

[56] References Cited

UNITED STATES PATENTS

|           |         |          |           |
|-----------|---------|----------|-----------|
| 2,099,743 | 11/1937 | Kroeger  | 252/175 X |
| 2,333,443 | 11/1943 | Robinson | 252/135   |
| 2,351,559 | 6/1944  | Treffler | 252/135   |
| 2,365,215 | 12/1944 | Rhodes   | 252/135 X |
| 2,515,880 | 8/1950  | MacMahon | 252/135   |
| 2,909,490 | 10/1959 | Metziger | 252/135   |
| 3,247,118 | 4/1966  | Matthaei | 252/99    |
| 3,285,859 | 11/1966 | Jelen    | 252/385   |

3,620,979 11/1971 Corliss et al. .... 252/385  
3,630,928 12/1971 Fuchs. .... 252/135

FOREIGN PATENTS OR APPLICATIONS

4,111 4/1912 Great Britain  
494,628 10/1938 Great Britain  
525,514 8/1940 Great Britain

Primary Examiner—Leon D. Rosdol

Assistant Examiner—P. E. Willis

Attorney, Agent, or Firm—William A. Skinner; Timothy Tinkler

[57] ABSTRACT

A method of preparing a particulate detergent builder includes admixing liquid sodium silicate with anhydrous soda ash having a particle size of less than 200 microns at a temperature between 21°-51°C., passing the resultant wetted granules through at least an eight mesh screen and rapidly heating the screened material to in excess of 100°C.

3 Claims, No Drawings

1  
**SILICATED SODA ASH****BACKGROUND OF THE INVENTION**

It is known to be desirable to incorporate alkali metal silicates into various detergent compositions both for their inherent detergency and for their ability to protect ceramic and reactive metal surfaces from corrosive attack. Various problems have presented themselves in attempting to effect this incorporation. The most readily available source of dry, granular soluble  $\text{SiO}_2$  is the crystalline sodium metasilicates which, however, are too alkaline for many uses and in any event tend to segregate from the compositions into which they are incorporated. Other particulate sodium silicates having a higher ratio of silica to sodium oxides are not readily available, thus being too expensive for incorporation into most detergent compositions. Furthermore, where used, the tendency of these particulate materials is again to segregate and/or contribute substantially to dusting. Various techniques have been suggested for blending liquid silicates into a detergent composition followed by drying to achieve the desired particulate state. However these methods, such as spray drying or agglomeration, generally require expensive equipment and hence large scale production to justify the necessary investment.

**STATEMENT OF THE INVENTION**

Therefore it is an object of the present invention to provide a method for incorporating liquid silicates into a detergent formulation.

It is a further object of the present invention to provide a particulate silicated soda ash and a method of preparing same.

There has now been found a method of preparing a free-flowing particulate detergent builder, which method consists essentially of:

- a. preparing an aqueous solution of sodium silicate having a  $\text{Na}_2\text{O}:\text{SiO}_2$  weight ratio of from 1:1.6 to 3.3 and a solids content of from 38 to 50 percent by weight;
- b. admixing said solution with a substantially anhydrous sodium carbonate having a particle size of less than about 200 microns, said carbonate constituting from 45 to 70 percent by weight of the mixture;
- c. maintaining the temperature during admixture between 21°-51°C.;
- d. after thorough admixing, passing the resultant material through at least an eight mesh screen;
- e. rapidly heating the wetted, screened material to a temperature within the range of 105° to 250°C. and,
- f. recovering as the product a substantially dry particulate detergent builder having a bulk density of from 25 to 50 pounds per cubic feet and a uniform  $\text{SiO}_2$  content of from 10 to 30 percent by weight.

In such a detergent builder the silicate is distributed uniformly on the soda ash particles and a sufficient amount of said silicate may be incorporated to provide the desired and advantageous properties. Further it has been found that the resultant particles are highly absorbent, being capable of taking up, for example, up to 15 percent of their weight of a liquid surfactant. It will be appreciated that the equipment requirements of one

desiring to produce such a detergent builder are quite modest. Hence, most any desired size production operation may be achieved.

**DESCRIPTION OF THE PREFERRED EMBODIMENTS**

The sodium silicate employed will generally be one of those commercially available which have an  $\text{Na}_2\text{O}:\text{SiO}_2$  weight ratio within the stated range of from about 1:1.6 to 3.3 and a solids content within the range of from 38-50 percent by weight, the balance being water. Of course it is possible to adjust the ratio of the solution to a desired point by the addition of sodium hydroxide. The amount of such a silicate employed will be within the range of from 30-55 percent of the combined aqueous silicate/soda ash, corresponding to a uniform  $\text{SiO}_2$  content in the final product within the range of 10 to 30, preferably 18-22, percent by weight.

20 The sodium carbonate must be substantially anhydrous since those materials having water bound thereto will not accept the desired quantities of silicate. That the soda ash has a particle size of less than about 200 microns, for example passing through an eighty mesh screen, has been found important to the process since otherwise a sticky mass, essentially impossible to mix while retaining a particulate form, will be obtained on addition of the silicate solution. The amount of sodium carbonate employed falls within the range of 45 to 70 percent by weight of the mixture.

It has been noted that during the admixture of the silicate and soda ash it is essential that the temperature be maintained within the range of 21° to 51°C. At lower temperatures the mixture becomes quite heterogeneous consisting of quantities of silicate coated with soda ash and "free" soda ash. On the other hand, at temperatures in excess of about 51°C. a taffy-like mass is formed which is unsuitable for the subsequent operations.

40 The result of the foregoing is a wet granular material which is then passed through at least an eight mesh screen in order to obtain a particle size suitable for subsequent operations. By the phrase "at least an eight mesh screen" it is intended to refer to an eight mesh screen (Tyler or U.S. Standard) or one the openings of which are smaller, e.g., a 10 mesh screen.

The thus-screened material is then passed to a heating step wherein the temperature is rapidly raised to within the range of 105° to 250°C. For example, the material being screened may be allowed to fall directly onto the surface of a hot plate having the appropriate temperature. The purpose of the heating step is to cause the formation of water vapor within the silicate and the subsequent release thereof, thereby resulting in the formation of a silicate "foam." Temperatures of less than 105°C. do not yield any substantial foaming, thus dictating a product having a bulk density higher than is generally desired for use as a detergent builder. While temperatures in excess of 250°C. may be used, no significant additional advantage is obtained, an optimum low bulk density being achieved at the stated temperature. Obviously then, control of the temperature within this range is one method of regulating the bulk density of the product within the stated range of 25 to 50, preferably 35 to 50, pounds per cu. ft.

60 It will be apparent from the foregoing that, with the appropriate choice of equipment, the process may be

operated either batch-wise, for small amounts with specific formulations, or, preferably, in a continuous manner.

A surprising result of this process, and characteristic of the product, is that the pH of the silicated soda ash is lower than that of either ingredient alone. For example, the pH (measured as a 1 percent aqueous solution) of a product made from sodium silicate having a ratio of 1:2.4 and containing 20 percent  $\text{SiO}_2$  is measured at 11.0. A solution of soda ash alone reads 11.4 and the silicate has a pH of 11.3.

In order that those skilled in the art may more readily understand the present invention and certain preferred embodiments by which it may be carried into effect, the following specific examples are afforded.

#### EXAMPLE 1

In the following Table the samples are prepared by adding the silicate to the soda ash over a period of 5 minutes while mixing at low speed in a Hobart mixer at a temperature of about 43°C. The soda ash employed is an anhydrous sodium carbonate, 98 percent of the particles of which pass through an 80 mesh Tyler sieve, indicating a particle size of less than 174 microns. Mixing is continued for 10 minutes after addition is completed, following which the wet granular material is screened through a 10 mesh Tyler sieve onto a hotplate having a surface temperature as indicated.

TABLE

| Sample | $\text{Na}_2\text{CO}_3$<br>(gms.) | Aqueous<br>Silicate<br>(gms.) | $\text{Na}_2\text{O}:\text{SiO}_2$<br>(wt. ratio) | Silicate<br>Solids<br>(%) | Drying<br>Tempera-<br>ture (°C.) | Product<br>$\text{SiO}_2$<br>(%) | Bulk<br>Density<br>(lbs./ft. <sup>3</sup> ) |
|--------|------------------------------------|-------------------------------|---------------------------------------------------|---------------------------|----------------------------------|----------------------------------|---------------------------------------------|
| 1      | 500                                | 450                           | 1:2.5                                             | 47.3                      | 110                              | 19-20                            | 45                                          |
| 2      | 500                                | 450                           | 1:2.5                                             | 47.3                      | 188                              | 19-20                            | 28                                          |
| 3      | 500                                | 450                           | 1:2.5                                             | 47.3                      | 438                              | 19-20                            | 26                                          |
| 4      | 560                                | 500                           | 1:3.22                                            | 38.3                      | 160                              | 19-20                            | 34                                          |
| 5      | 600                                | 500                           | 1:2.84                                            | 43.1                      | 160                              | 19-20                            | 35                                          |
| 6      | 530                                | 500                           | 1:2.0                                             | 44.1                      | 160                              | 19-20                            | 34                                          |
| 7      | 510                                | 548                           | 1:1.6                                             | 43.6                      | 160                              | 19-20                            | 36                                          |
| 8      | 500                                | 255                           | 1:2.0                                             | 44.1                      | 182                              | 12                               | 34                                          |

By comparing Samples 1, 2 and 4 of the Table, the effect of temperature in the drying step on the bulk density of the product can be seen. Further, Sample 3 indicates that an additional and substantial temperature increase has essentially no further effect on the ultimate bulk density. Sample 8 was determined to be capable of absorbing up to 15 percent of a liquid polyethoxy ether nonionic surfactant while still remaining free-flowing.

#### EXAMPLE 2

By way of comparison, Sample 3 is repeated, substituting a commercially available anhydrous sodium carbonate, 95 percent of the particles of which pass through a 30 mesh screen, 92 percent being retained on a 100 mesh screen. Upon addition of the silicate, a sticky mass not capable of being converted into a uniform granular mixture is obtained. This experiment is repeated substituting a second commercial soda ash, 95 percent of which is retained on a 100 mesh screen, with the same results.

Upon grinding the first of the aforesaid commercial soda ashes until it passes through an eighty mesh screen, a satisfactory product similar to Sample 3 is obtained.

#### EXAMPLE 3

Sample 3 is repeated, this time conducting the mixing operation at a temperature of 18°C. The result is a heterogeneous mixture containing granules of silicate coated with soda ash and about 20 percent of silicate-free soda ash. Conducting the same experiment at a temperature just in excess of 51°C., a taffy-like mass unsuitable for further processing is obtained.

While the invention has been described with reference to certain preferred embodiments thereof, it is not to be so limited since changes and alterations may be made therein while remaining within the intended scope of the appended claims.

I claim:

15. 1. A method of preparing a free-flowing particulate silicated sodium carbonate detergent builder which method consists essentially of:
- preparing an aqueous solution of sodium silicate having an  $\text{Na}_2\text{O}:\text{SiO}_2$  weight ratio of from 1:1.6 to 20 3.3 and a solids content of from 38-50 percent by weight;
  - admixing said solution with substantially anhydrous sodium carbonate having a particle size of less than about 200 microns, said carbonate constituting from 45 to 70 percent of the mixture;
  - maintaining the temperature during admixture between 21° and 51°C.;
  - after thorough admixing, passing the resultant ma-

terial through at least an eight mesh screen;

- rapidly heating the screened material to a temperature within the range of 105° to 250°C. and,
- recovering as the product a substantially dry particulate detergent builder having a bulk density of from 25 to 50 pounds per cu. ft. and a uniform  $\text{SiO}_2$  content from 10 to 30 percent by weight.

2. The particulate free-flowing silicated sodium carbonate detergent builder produced by the method of claim 1 which is a substantially anhydrous coherent mixture of sodium carbonate and a sodium silicate having a  $\text{Na}_2\text{O}:\text{SiO}_2$  ratio of 1:1.6 to 3.3, the amount of  $\text{SiO}_2$  being within the range of 10 to 30 percent, said builder having a bulk density within the range of 25 to 50 lbs./ft.<sup>3</sup>, being capable of absorbing up to 15 percent of its weight of a liquid nonionic surfactant and having a pH lower than that of either the sodium silicate or sodium carbonate from which it is formed.

3. The particulate free-flowing silicated sodium carbonate detergent builder produced by the process of claim 1 containing from 18 to 22 percent by weight  $\text{SiO}_2$ , as sodium silicate having a  $\text{Na}_2\text{O}:\text{SiO}_2$  weight ratio 1:2.4, said builder having a bulk density within the range of 35 to 50 lbs./ft.<sup>3</sup>, being capable of absorbing about 15 percent of its weight of a liquid nonionic surfactant and having a pH, measured as a 1 percent aqueous solution, of about 11.0.

\* \* \* \* \*